

B. BART.

ELECTROLYTIC REFINING OF METALS.  
APPLICATION FILED DEC. 12, 1917.

1,295,100.

Patented Feb. 25, 1919.



Fig. 1.



Fig. 2.

INVENTOR.  
*Blasius Bart*  
BY  
*Macdonald Macdonald*  
his ATTORNEYS

# UNITED STATES PATENT OFFICE.

BLASIUS BART, OF NEWARK, NEW JERSEY.

## ELECTROLYTIC REFINING OF METALS.

1,295,100.

Specification of Letters Patent. Patented Feb. 25, 1919.

Application filed December 12, 1917. Serial No. 206,740.

To all whom it may concern:

Be it known that I, BLASIUS BART, a citizen of the Republic of Switzerland, residing at 231 North 7th street, in the city 5 of Newark, in the county of Essex and State of New Jersey, have invented certain new and useful Improvements in Electrolytic Refining of Metals, of which the following is a full, clear, and exact specification, such as will enable others skilled in the art to which it appertains to make and use the same.

My present invention relates to a novel process for depositing metals electrolytically and incidentally to a novel process 15 of preparing anodes for this purpose, as well as to an improved anode and anode core.

In electro-plating work it is essential, 20 among other things, that the surfaces of the anodes which yield the metal to the electrolyte or both should be composed of metal as nearly pure as possible, and for this reason anodes are often prepared from 25 metal electrolytically deposited. In plating with copper, for instance, it has been customary to deposit the copper from a relatively impure copper anode upon a thin plate used as a cathode. The copper thus 30 deposited is brittle and granular but quite pure. It is not tenacious enough to be relied upon in use as an anode for the final process of electro-plating, and it is therefore customary to melt and roll it to 35 form new plates fit for use.

The anode plates so made are generally suspended by hooks connected in the plating circuit and passing through openings near the top of the plates, and the plates so 40 suspended are immersed in the electrolyte.

It is found in practice that, when plates are used as anodes in this manner, they waste away rapidly at their lower and side edges so that they diminish rapidly in effective area, often breaking off so that pieces 45 of copper (or other metal as the case may be) drop uselessly to the bottom of the cell.

The result is that a useless stump of waste metal of irregular shape is left suspended 50 from the hooks, which has to be melted up as scrap. This wastage is due to the fact that the solution of the anode metal in the electrolyte is far more rapid at the edges of the plate, where the liquid has a chance 55 to circulate, than at other parts of the plate,

and that, for this reason, the plate is rapidly eaten away in the manner above described.

It is the principal object of my present invention to provide a process of preparation and use of the anode, as well as a form 60 of anode and core therefor, whereby the above objections are obviated, and whereby the entire supply of metal used in plating is evenly consumed, leaving no stump or wastage. By the employment of my process 65 I obtain the further advantage of doing away with the necessity of melting and rolling the electrolytic metal preparatory to using it in the final process of electroplating. This object is attained by reason of 70 the fact that my novel form of core makes it possible to obtain at once a smooth, even and tenacious surface, instead of the granular, brittle and unreliable surface obtained 75 by the older method of preparation.

In the accompanying drawings, Figure 1 is a face view or elevation of one of my anode plates with a portion of the plating metal removed to show the core, and Fig. 2 is a sectional view of the same on the line 80 2-2 of Fig. 1.

In my improved process I employ a core alternately on the negative and positive poles of the plating cell, and this core has a novel construction which forms a part 85 of the subject matter of my present invention.

This core A is in the form of a grid, wherein the openings are of a considerable size, so as to allow a large deposit of metal 90 around their edges without their being stopped up. In the form shown this grid is formed of elements B, preferably lenticular in shape, and connected by necks C. These parts form the borders of openings 95 D which are preferably at least about as large as the elements B. In order to suspend these grids in the electrolyte I provide them with hooks E which can be hung over the positive or negative wires in a 100 well known manner.

For obvious reasons I prefer to make these grids or cores of a metal which will not be attacked by the particular electrolyte intended to be used. Any suitable metal may be 105 used as will be understood by those skilled in the art, and it is not necessary that it should be as good a conductor as the metal to be plated with.

In carrying out my improved process I 110

first use the core A as a cathode, the anode being made of the metal intended to be plated with, as in the preparation of pure electrolytic metal by the older processes. 5 The difference is that I have found that, by the use of my improved core, the deposited metal is generally smooth instead of granular, and is sufficiently tenacious and reliable for immediate use as an anode, without being melted and rolled. This is due to the 10 fact that the form of the core A is highly favorable to circulation of the fluid; and, presenting as it does, a very extended aggregate of edges in proportion to face area, 15 there is a much more uniform action over the entire core than would be the case if it were a plate with few or no perforations.

In consequence of this action, the preliminary electrolytic operation builds up a body 20 of pure metal to be plated as shown at F, which is in the best possible condition to serve as an anode in the final process of plating. As shown in the lower and left hand side of Fig. 1, the deposition of metal during this preliminary process should not be 25 carried so far as to close the openings D entirely. Indeed, in many cases a larger proportion of open area than shown may be used in the anode.

30 I have found in practice that, where a composite body prepared as just described is used as an anode the deposited metal is consumed evenly over the whole surface until entirely consumed, owing to the large 35 area of perforation or open space, and the consequent great extension of the edges in proportion to face area. It will also be

noticed that, owing to the openings growing larger as the plating metal is consumed, there is practically no diminution of total 40 area exposed to the bath, thereby contributing to uniformity in the internal resistance of the bath.

By use of my core and of my process I not only avoid the expense of the older methods 45 of preparation, but I have no wastage and no dropping of pieces to the bottom of the cell. The final plating, too, is smooth, even and lasting.

What I claim is—

1. In the art of electroplating with metal depositing metal electrolytically upon an anode core composed of solid portions alternating with openings to prepare the metal for final deposition and then using the composite 55 body so formed as an anode.

2. In the art of electroplating with metal, depositing metal electrolytically upon a core composed of elements and connecting necks bordering open spaces of areas not greatly 60 smaller than the areas of said elements until said open spaces are partly closed and then employing the composite body so produced as an anode in the final plating.

3. A core for the purpose described composed of elements and connecting necks limiting open spaces not greatly less in area than said elements.

4. A composite body composed of a core of the character set forth in claim 3 hereof and covered with electrolytically deposited metal in quantity insufficient to close the openings in the grid.

BLASIUS BART.